

## 1

3,281,203

## MODIFICATION OF THE DYEING CHARACTERISTICS OF ISOTACTIC POLYOLEFIN FIBERS CONTAINING BASIC NITROGEN GROUPS THROUGH TREATMENT WITH A DIEPOXIDE PRECURSOR AND AN ALKALINE CATALYST

Ubaldo Riboni, Milan, and Luigi Bartolucci, Terni, Italy, assignors to Montecatini Società Generale per l'Industria Mineraria e Chimica, Milan, Italy, a corporation of Italy

No Drawing. Filed June 12, 1962, Ser. No. 201,818  
Claims priority, application Italy, June 15, 1961, 11,056  
16 Claims. (Cl. 8—115.5)

The present invention relates to a process for improving the dyeing characteristics of textile fibers obtained by the extrusion of mixes containing:

(A) polyolefin prepared with stereo-specific catalysts, and exhibiting a high content of crystallinity due to the isotactic structure.

(B) a basic nitrogen-containing compound.

The invention also encompasses the improved products obtained from this process.

Processes for improving the dye receptivity of textile fibers to different classes of dyes, especially to acid dyes, by the extrusion of mixtures containing crystalline polyolefins with 1-25% by weight based on the polyolefin, of polymeric basic nitrogen-containing products, have been described in commonly assigned United States applications.

Methods have also been described, in commonly assigned applications, for further improving the dyeing characteristics, particularly the fastness of the thus obtained polyolefinic fibers, by means of treatments with diepoxydic compounds, particularly with aqueous solutions of ethyleneglycol diglycidyl ether or diglycidyl ether.

We have now surprisingly found that remarkably better results are obtained when the fibers obtained from the mixes mentioned above are treated with chlorohydrins and alkaline agents such as sodium hydroxide or potassium hydroxide and the like, which form the corresponding diepoxydic compounds at the moment of use or, even more desirably, to operate so that the diepoxydic formation occurs directly on the fiber.

The dichlorohydrins are employed in aqueous solutions dissolved in organic solvents such as aliphatic, aromatic hydrocarbons, etc., or in the anhydrous state.

The alkaline agent is added directly to the vessel or apparatus wherein the treatment of the fibers is carried out, either immediately before or after the introduction of fibers into the vessel.

The treatment of the yarns is performed before and/or after their stretching, for times which may vary from a few (at least 30) seconds to 2-3 hours, and at temperatures varying from room temperature to 10° below the melting point of the polymer. The alkaline agent, e.g. sodium hydroxide, is added to the solution of dichlorohydrin in the amount stoichiometrically needed for conversion to the diepoxydic. Dichlorohydrin may be employed either in the pure form or while containing the normal impurities.

The following examples are given to better illustrate the present invention without limiting its scope.

All parts and proportions are by weight unless otherwise indicated.

## 2

## Example 1

The dichlorohydrin of ethyleneglycol diglycidylether



is prepared by introducing 64 g. (1 mole) of ethyleneglycol and 0.4 cc. of boron trifluoride in 45% ethereal solution into a three-necked 500-cc. flask, provided with thermometer, stirrer and reflux condenser. The mass is warmed up to 90° C. and 185 g. epichlorohydrin are added within two hours. The mass is kept in reaction for one additional hour, and then is cooled to room temperature.

The dichlorohydrin thus obtained, which has a titer of about 72%, is ready for use.

A yarn obtained by the melt spinning of a mix comprising 95% of polypropylene prepared with stereospecific catalysts ( $[\eta]^1=1.51$ , ash content=0.028%, residue to heptane extraction=95.6%) and 5% of octadecylamine/epichlorohydrin/piperazine condensate, is immersed for 5 minutes at 25° C. in a 5% aqueous solution of the dichlorohydrin of ethyleneglycol diglycidylether, to which 13 g. of NaOH per liter of solution have been added immediately before. After a treatment with squeezing rolls, about 70% of the solution remains on the yarn. The yarn is then subjected to a thermal treatment at 120° C. for 20 minutes.

The treated yarn is dyed with the following dyes:

30 Alizarine yellow 2 G (C.I. #14025) (C.I. mordant yellow 1) (acid)  
Red for wool B (C.I. #27200) (C.I. acid red 115) (acid)  
Alizarine red S (C.I. #58005) (C.I. mordant red 3) (acid)  
35 Alizarine blue SE (C.I. #63000) (C.I. acid blue 43) (acid)  
Acid black JVS (C.I. #20470) (C.I. acid black 1) (acid)  
Setacetyl bright blue BG (C.I. #61505) (C.I. disperse blue 3) (plastosol)

40 The dyeings are carried out by maintaining the yarn in the bath containing 2.5% dye, based on the weight of fiber, at a fiber/bath ratio of 1:40.

The dyeings with acid dyes are carried out in the presence of 3% ammonium acetate (based on the weight of fiber) and 1% of a surfactant prepared by the condensation of ethylene oxide with p.cresol. 30 minutes after the boiling commences, 2%, based on the weight of fiber, of a 10% acetic acid solution is added in order to improve the rate of utilization of the bath.

Dyeings with plastosoluble (dispersed) dyes are carried out in the presence of 2% (based on the fiber weight) of a surfactant. The yarns, after dyeing, are rinsed with running water and are intensely dyed, either with the acid or plastosoluble dyes. The light, washing and friction fastness of these dyed yarns is shown to be entirely satisfactory.

## Example 2

The yarn of Example 1 is passed through a bath containing 100 g./l. of the dichlorohydrin of ethyleneglycol diglycidylether and 26 g./l. of NaOH which is prepared immediately before the addition of the fiber. The feeding rate of the yarn is 10 m./minute and the bath tempera-

1 Here and in the following examples the intrinsic viscosity has been measured in tetralin at 135° C.

ture is 30° C. The yarn is allowed to remain in the epoxidation bath for 2 minutes. The roving is allowed to pass between rolls so that 2% of the pure epoxide is allowed to remain on the yarn. The collected roving is treated in an autoclave with steam at 120° C. for 1 hour. The yarn, upon being dyed with the dyes of Example 1, gives intense, fast colors.

*Example 3*

A yarn obtained by the melt spinning of a mix containing 95% polypropylene prepared with stereospecific catalysts ( $[\eta]=1.51$ , ash content=0.028%, heptane extraction residue=95.6%) and 5% of an octadecylamine/epichlorohydrin/piperazine condensate is immersed for 5 minutes at 40° C. in a 6% aqueous solution of the dichlorohydrin of ethyleneglycol diglycidylether. An amount of sodium hydroxide corresponding to 80% of the theoretical amount based on the dichlorohydrin is then added. The mass is finally centrifuged, treated with warm water and dried. The treated yarn gives intense, fast colors upon being dyed with the dyes of Example 1.

*Example 4*

A yarn obtained through the melt spinning of a mix containing 95% of polypropylene prepared with stereospecific catalysts ( $[\eta]=1.51$ , ash content=0.028%, heptane extraction residue=95.6%) and 5% of dichloroethane/hexamethylendiamine condensate is immersed for 10 minutes, at 20° C., in a 3% aqueous solution of the dichlorohydrin of ethyleneglycol diglycidylether. Then an amount equivalent to the sodium hydroxide used in Example 3 is added. The mass is centrifuged, heated in autoclave at 120° C. for one hour and then washed with water and dried. The treated yarn gives intense, fast colors upon being dyed with the dyes of Example 1.

*Example 5*

A yarn obtained by the melt spinning of a mix containing 95% of polypropylene prepared with stereospecific catalysts ( $[\eta]=1.51$ , ash content=0.028%, heptane extraction residue=95.6%) and 5% of octadecylamine/epichlorohydrin/hexamethylendiamine condensate is immersed for 30 minutes at 60° C. in a 3% aqueous solution of the dichlorohydrin of ethyleneglycol diglycidyl-ether.

Then sodium hydroxide is added as in Example 4. The mass is then treated in hot air at 130° C. for 20 minutes, washed with water and dried. The treated yarn yields intense and fast colors upon being dyed with the dyes of Example 1.

*Example 6*

A yarn obtained by the melt spinning of a mix containing 95% of polypropylene prepared with stereospecific catalysts ( $[\eta]=1.51$ , ash content=0.028%, heptane extraction residue=95.6%) and 5% of isotactic crystalline poly-2-vinylpyridine ( $[\eta]=0.22$ ) is immersed for 40 minutes at 40° C. in a 10% aqueous solution of the dichlorohydrin of ethyleneglycol diglycidylether.

Then stoichiometrically equivalent amounts of sodium hydroxide are added. The mass is centrifuged, treated in hot air at 130° C. for 30 minutes, washed with water and dried. The treated yarn gives intense, fast colors upon being dyed with the dyes of Example 1.

*Example 7*

2000 cc. of monochloroglycerol and 5 cc. of a 45% ether solution of boron trifluoride are poured into a 3-liter, three-necked flask, provided with reflux condenser, thermometer and tap funnel. The mixture is heated at 95-100° C. and 610 cc. of epichlorohydrin are added over a period of about two hours so as to keep the temperature constant. When these additions are completed, the flask is kept at 95-100° C. for two additional hours

and the excess monochloroglycerol is distilled off under vacuum.

Then the dichlorohydrin of the formula:



is collected at 150-165° C. under 3 mm. pressure. The yield of pure dichlorohydrin is higher than 80%.

10 A 40% aqueous solution of this dichlorohydrin is prepared and treated with an amount of NaOH solution equivalent to the theoretical amount required. A roving of the yarn obtained following the procedure of Example 1 is passed into this solution immediately. After a squeezing between rolls so as to leave on the yarn about 2% pure diglycidylether, the yarn is treated with a stream of hot air at 130° C. for 15 minutes. The colors obtained upon dyeing these yarns with the acid dyes of Example 20 1, after the epoxidic treatment, are fast and bright.

Many variations and modifications can, of course, be practiced without departing from the spirit and scope of the present invention.

Having thus described the invention, what it is desired to secure and claim by Letters Patent is:

1. A process for improving the dyeing characteristics of fibrous materials such as filaments and yarns obtained by the extrusion of mixes of a polyalpha-olefin exhibiting a high content of crystallinity due to isotactic structure and 1-25%, based on the weight of said polyolefin, of a polymeric basic-nitrogen containing compound, which process comprises contacting the fibrous materials in a bath with a glycol dichlorohydrin and a stoichiometric amount of a strong inorganic base to convert said dichlorohydrin into diepoxide, at temperatures between room temperature and 10° C. below the softening point of the polymer, for a time varying from 30 seconds to 3 hours.
2. The process of claim 1 wherein the fibrous materials are successively contacted in said bath with the glycol dichlorohydrin and the strong inorganic base.
3. The process of claim 1 wherein the fibrous materials are simultaneously contacted in said bath with the glycol dichlorohydrin and the strong inorganic base.
4. The process of claim 1 wherein the polymer exhibiting a high content of crystallinity due to isotactic structure is polypropylene.
5. The process of claim 1 wherein the polymeric basic-nitrogen containing compound is selected from the group consisting of octadecylamine-epichlorohydrin-piperazine condensates, octadecylamine-epichlorohydrin-hexamethylendiamine condensates, isotactic crystalline polyvinyl pyridines and dihalogen derivative-diamine condensates.
6. The process of claim 1 wherein the glycol dichlorohydrin is the dichlorohydrin of diglycidylether.
7. The process of claim 1 wherein the glycol dichlorohydrin is the dichlorohydrin of the ethyleneglycol diglycidylether.
8. The process of claim 1 wherein the strong inorganic base is sodium hydroxide.
9. The process of claim 1 wherein the glycol dichlorohydrin is in the anhydrous state.
10. The process of claim 1 wherein the glycol dichlorohydrin is in aqueous solution.
11. The process of claim 1 wherein the glycol dichlorohydrin is dissolved in an organic solvent.
12. The process of claim 1 wherein the fibrous materials are contacted with the glycol dichlorohydrin and the strong inorganic base before stretching thereof.
13. The process of claim 1 wherein the fibrous materials are contacted with the glycol dichlorohydrin and the strong inorganic base after stretching thereof.
14. The process of claim 1 when carried out in a batchwise manner.
15. The process of claim 1 when carried out in a continuous manner.

16. Fibrous materials possessing improved dyeing characteristics selected from the group consisting of filaments and yarns, when obtained according to the process of claim 1.

|           |         |                  |       |         |
|-----------|---------|------------------|-------|---------|
| 2,998,295 | 8/1961  | Goldann          | ----- | 8—115.5 |
| 3,013,998 | 12/1961 | Battaglioli      |       |         |
| 3,098,697 | 7/1963  | Cappuccio et al. | ----- | 8—55 X  |
| 3,107,228 | 10/1963 | Cappuccio et al. | ----- | 8—55 X  |
| 3,151,928 | 10/1964 | Cappuccio et al. | ----- | 8—115.5 |
| 3,223,472 | 12/1965 | Monaci et al.    | ----- | 8—115.5 |

**References Cited by the Examiner**

UNITED STATES PATENTS

|           |        |           |       |         |
|-----------|--------|-----------|-------|---------|
| 2,730,427 | 1/1956 | Suen      | ----- | 8—116   |
| 2,903,381 | 9/1959 | Schroeder | ----- | 8—116 X |
| 2,985,501 | 5/1961 | Gagarine  | ----- | 8—120   |

NORMAN G. TORCHIN, *Primary Examiner.*

JULIAN S. LEVITT, *Examiner.*

J. CANNON, *Assistant Examiner.*